

## UNITED STATES PATENT OFFICE

CAMILLE DREYFUS, OF NEW YORK, N. Y.

## WARP PRINTING

No Drawing.

Application filed September 8, 1928. Serial No. 304,803.

This invention relates to the production of novel color effects by the printing of warps of yarns of organic derivatives of cellulose.

An object of my invention is to locally color 5 warps of yarns of organic derivatives of cellulose, whereby novel color effects are produced. Other objects of my invention will appear from the following detailed description.

10 In the weaving of fabrics, a warp is first made which comprises a series of parallel yarns wound on a beam. This warp is fed to a loom where the weft or filling is woven in to make a fabric. When yarns of organic 15 derivatives of cellulose are employed in the warp, it is necessary to size the same in order to impart sufficient strength to the warp to withstand the drastic conditions to which it is subjected in the loom.

20 I have made the surprising discovery that such warps, while they have the size thereon, may be successfully printed with a suitable printing paste despite the presence of the size thereon.

25 In accordance with my invention, I locally color warps of yarns containing organic derivatives of cellulose which have thereon a suitable size, by locally applying thereto a coloring matter.

30 The warps to be locally colored by my invention are parallel yarns wound on a beam corresponding in length to the width of the fabric eventually to be made therefrom. In order to prevent the warp from becoming 35 disarranged during printing, leases are preferably woven at intervals therein. The warp may consist of yarns of organic derivatives of cellulose, examples of which are organic esters of cellulose such as cellulose acetate, 40 cellulose formate, cellulose propionate and cellulose butyrate and cellulose ethers such as ethyl cellulose, methyl cellulose and benzyl cellulose. If desired the warp may also contain yarns of other fibres such as silk, cotton, 45 ton, reconstituted cellulose, wool or flax.

The warp yarns are sized with a suitable size which may contain glue, gelatin, starches, dextrines, etc. or any suitable mixtures of these, in order to increase the strength of such yarns. The sized yarns then have locally applied thereto a suitable coloring matter, 50 in any suitable manner. The colored designs may be applied by printing with engraved or embossed rolls or blocks, or it may be applied by brushing or spraying of a suitable coloring material onto stencils placed over the warp.

The dyestuffs employed in the coloring matter may be any suitable dye that has an affinity for organic derivative of cellulose 60 yarns. Examples of such dyestuffs are insoluble anthraquinone dyes in the unreduced state dispersed in aqueous dispersions by means of a dispersing medium such as Turkey red oil. Other suitable dyes such as the basic dyes may also be employed. The coloring matter also contains suitable thickeners such as gum arabic, gum tragacanth, British gum, dextrine, starches, etc.

65 After the coloring matter is applied locally to the warps, they may be dried on rotating heated drums or cans or in any other suitable manner, and, if desired, they may be steamed or aged. The warps, when treated in the above manner, are ready for 70 weaving and may be woven with a weft or filling of yarns of organic derivatives of cellulose or of other fibres such as silk, cotton, etc. The filling yarn may be of any desired color.

75 An advantage of my process is due to the fact that the thickener of the printing paste, when it is retained on the warp, further increases the strength of the same and acts as a size during the weaving operation. Instead of weaving the warp to make a woven fabric, the warp may be knitted to form a 80 warp knitted fabric.

85 After weaving or knitting of the printed warp, a fabric is produced having subdued 90

local color effects. This effect is produced by having the color of the weft blending with the well defined color pattern of the original warp. By this method a fabric is produced having colored designs, the outlines of which are not sharp.

In order further to illustrate my invention the following specific example is given without limiting the scope thereof.

10

*Example*

A warp is employed that consists of parallel yarns made of cellulose acetate and having leases woven therein at intervals of, say one yard, to retain the warp in place during printing. The warp yarns are sized prior to beaming with an appropriate size containing gelatin, glycerine, castor oil and water. The warp is fed to an ordinary printing machine, where it is printed by means of suitable engraved rolls with a printing paste that is ordinarily used for printing fabrics containing cellulose acetate yarn.

An example of such printing paste is:

25

|                           | Parts by weight |
|---------------------------|-----------------|
| Basic dyestuff            | 10 to 50        |
| Acetic acid (40%)         | 25              |
| Ethyl alcohol             | 25 to 30        |
| Diacetin                  | 25              |
| Water                     | 265 to 250      |
| Gum arabic solution (50%) | 650 to 620      |

The printed warp is then dried by being passed around rotating heated drums or cans, and if desired, may be aged by steaming. The warp is now ready for weaving and this is done in any suitable loom after the leases have been removed. The weft or filling may be a yarn of organic derivatives of cellulose or of any other fibre and may be of any desired color. Despite the presence of the size on the warp yarns, the printing paste produces clear and well colored designs thereon.

45 It is to be understood that the foregoing detailed description is given merely by way of illustration and that many variations may be made therein without departing from the spirit of this invention.

50 Having described my invention, what I claim and desire to secure by Letters Patent is:

1. In the method of producing warp print effects, the step of printing a warp containing organic derivative of cellulose yarns and having a size thereon, with a paste containing an insoluble anthraquinone dye.

2. In the method of producing warp print effects, the step of printing a warp containing cellulose acetate yarns and having a size thereon, with a paste containing an insoluble anthraquinone dye.

3. The method comprising passing a warp of cellulose acetate yarn having leases at intervals therein, which yarn has a size con-

taining gelatin thereon, in contact with a rotating printed roll which applies a printing paste containing an insoluble anthraquinone dye locally thereto, passing the warp over drying drums and then converting said warp into a fabric.

In testimony whereof, I have hereunto subscribed my name.

CAMILLE DREYFUS.

75

80

85

90

95

100

105

110

115

120

125

130